

Nov. 28, 1950

K. H. BRANDT

2,531,389

METHOD OF MAKING CAPACITORS

Filed July 28, 1944

8 Sheets-Sheet 1



INVENTOR.  
KRISTIAN H. BRANDT

BY *William D. Hall*

ATTORNEY

Nov. 28, 1950

K. H. BRANDT

2,531,389

METHOD OF MAKING CAPACITORS

Filed July 28, 1944

8 Sheets-Sheet 2

FIG. 3.



FIG. 4.



FIG. 5.



INVENTOR.  
KRISTIAN H. BRANDT

BY *William D. Hall*

ATTORNEY

Nov. 28, 1950

K. H. BRANDT

2,531,389

METHOD OF MAKING CAPACITORS

Filed July 28, 1944

8 Sheets-Sheet 3

FIG. 6.



FIG. 7.



FIG. 8.



INVENTOR.  
KRISTIAN H. BRANDT

BY *William D. Hall*

ATTORNEY

Nov. 28, 1950

K. H. BRANDT

2,531,389

METHOD OF MAKING CAPACITORS

Filed July 28, 1944

8 Sheets-Sheet 4



FIG. 9.



FIG. 10.

INVENTOR.  
KRISTIAN H. BRANDT

BY *William D. Hall*

ATTORNEY

Nov. 28, 1950

K. H. BRANDT

2,531,389

METHOD OF MAKING CAPACITORS

Filed July 28, 1944

8 Sheets-Sheet 5



FIG. 11.



FIG. 12.

INVENTOR.  
KRISTIAN H. BRANDT

BY *William D. Hall*

ATTORNEY

Nov. 28, 1950

K. H. BRANDT  
METHOD OF MAKING CAPACITORS

2,531,389

Filed July 28, 1944

8 Sheets-Sheet 6

FIG. 13.



Nov. 28, 1950

K. H. BRANDT

2,531,389

## METHOD OF MAKING CAPACITORS

Filed July 28, 1944

8 Sheets-Sheet 7



INVENTOR.  
KRISTIAN H. BRANDT

BY William F. Hall

**ATTORNEY**

Nov. 28, 1950

K. H. BRANDT

2,531,389

METHOD OF MAKING CAPACITORS

Filed July 28, 1944

8 Sheets-Sheet 8

FIG. 15.



FIG. 16.



FIG. 17.



FIG. 18.



FIG. 19.



INVENTOR.  
KRISTIAN H. BRANDT

BY *William D. Hall*

ATTORNEY

## UNITED STATES PATENT OFFICE

2,531,389

## METHOD OF MAKING CAPACITORS

Kristian H. Brandt, Red Bank, N. J.

Application July 28, 1944, Serial No. 547,094

2 Claims. (Cl. 29—25.42)

(Granted under the act of March 3, 1883, as  
amended April 30, 1928; 370 O. G. 757)

1

The invention described herein may be manufactured and used by or for the Government for governmental purposes, without the payment to me of any royalty thereon.

The present invention relates to capacitors and methods and apparatus for making the same.

Fixed capacitors are ordinarily made up in two forms. One comprises a stack of plates of metal conducting foil, separated by thin sheets of dielectric material, alternate layers of conducting foil being electrically joined. The other comprises two long strips of metal conducting foil, separated by dielectric material and rolled together so that one edge of one strip of foil is exposed for electrical connection at one end of the roll, and the opposite edge of the other strip is similarly exposed at the other end of the roll. In the present specification I will describe my invention in connection with the said two forms of fixed capacitors, but it is to be understood that the invention need not be limited thereto.

A good capacitor dielectric should be usable in very thin sheets so that capacitors may be made having relatively high capacity for their size. To be well suited to high frequency circuits, it should have a high dielectric strength to preclude it against puncture and resultant shorting of the capacitor, a low power factor and a relatively fixed dielectric constant over a wide frequency spectrum.

Although certain types of glass or vitreous enamel (which terms will be used interchangeably herein) have excellent dielectric characteristics, to my knowledge they have never been successfully used as interplate insulation in fixed capacitors prior to my invention. I have worked out a method of using such dielectrics so that the finished capacitors not only are as satisfactory as capacitors in general use, but I find that they are unexpectedly far superior. One possible deterrent to the use of glass or vitreous enamel as a capacitor dielectric has been that processes had not previously been evolved for quantity production so as to allow fabrication of such capacitors of a quality or at a cost to compete with other conventional capacitors.

Recently, largely in view of shortages in certain critical materials, such as mica, it has become increasingly important to find means of using alternate materials in capacitor production.

Extensive use of electrical and electronic equipment in motor vehicles and aircraft has also put additional requirements upon capacitors, such as substantial immunity to temperature changes, except in a predetermined manner, and insensitivity to vibration.

2

It is, therefore, an object of the present invention to provide capacitors, which will have a high ratio of capacitance to size, which will not be deleteriously affected by extremes of temperature or humidity or sudden fluctuations in temperature or humidity, and which will not be adversely affected by vibration incident to vehicular and aircraft installation.

Another object has been to incorporate into 10 a capacitor a dielectric which has good mechanical and electrical stability, a low power factor, a high dielectric strength and a high inherent insulation resistance.

It is a further object of the present invention 15 to provide a capacitor which is hermetically sealed against moisture, oil, dirt and the like so that it is protected against climatic changes, corrosion, etc.

Another object is to provide a capacitor which 20 is made of materials which are impervious to deterioration with time and which will form a single unitary structure, the parts of which will not separate even under exacting conditions.

A still further object of this invention is to 25 provide a capacitor in which the parts are retained in their relative positions mechanically and are not dependent upon fillers, such as wax or other filling compounds frequently used.

Still another object has been to design 30 capacitors which do not include strategic materials and which, in electrical and mechanical characteristics, are superior to, or at least compare favorably with, capacitors using strategic materials.

Another object has been to provide apparatus 35 and methods of manufacture for quantity production of such capacitors so as to allow their fabrication upon a practical basis and at a reasonable cost.

I have accomplished the foregoing by designing 40 capacitors utilizing glass or vitreous enamel as their dielectric material which is applied in liquid or paste form and, in some embodiments, metallic conducting plates which are similarly applied in liquid or paste form and by devising methods and means for handling such materials

45 and parts during the various manufacturing steps. The application of either the dielectric material or the conducting material, as the case 50 may be, in paste or liquid form, may be accomplished by any of several methods. Although I will describe the methods of spraying and dipping, the methods of painting with a brush or applying with a squeegee, preferably through a screen, or pressing, as with a rotary press, may 55 also be used. However, I do not wish to be limited

to these methods as my invention may be practiced by dispersing the said materials in other suitable manners.

One of the characteristics of glass or vitreous enamel, which makes it particularly valuable as a dielectric material for capacitors, is the fact that it can be produced in extremely thin films, such as of the order of .0015 to .005 inch in thickness without suffering the loss of its excellent dielectric characteristics. Likewise, the metallic conducting plates, which are applied in paste or liquid form, can be of the order of .0007 to .00175 inch in thickness. Of course, the materials may be used in my capacitors in thicknesses greater or less than those mentioned, but I believe that they result in eminently satisfactory practical capacitors which have extremely good electrical and mechanical characteristics and are well suited to replace capacitors using mica or paper dielectric, even were there no shortages of these materials.

Although the application of my invention may be varied to meet different requirements, in the present specification I shall illustrate my fundamental concepts by setting forth several preferred embodiments and processes covering the manufacture of both stacked type and rolled type capacitors.

I shall refer hereinafter to "green" vitreous enamel or glass to indicate that stage of its manufacture when it has attained sufficient viscosity and freedom from moisture so that it will not flow, but so that it may nevertheless be bent and handled without cracking and so that it may be readily cut. This green stage may be achieved by a preliminary partial heating or baking, in order to partially dry the enamel, after it has been dispersed in a thin film.

In the drawings appended thereto, some of the dimensions, particularly the thickness of some of the extremely thin elements, will be exaggerated for the purpose of clarity.

In the accompanying drawings, Figures 1 through 7 show steps in the manufacture of stacked type capacitors wherein metallic conducting material, applied in paste or liquid form, is used for the plates, Figures 8 through 12 show steps in the manufacture of stacked type capacitors wherein metal foil is used for the plates and Figures 13 through 19 show steps in the manufacture of rolled type capacitors wherein metal foil is used.

More specifically, Figure 1 is a perspective view showing the steps of spraying metallic material, in liquid form, through a spraying shield, onto a thin ribbon of vitreous enamel and then cutting the same, as indicated by the broken lines, into blanks, each blank comprising a rectangular sheet of vitreous enamel dielectric and a paddle-shaped plate of metallic, electrical conducting material.

Figure 2 is a perspective view showing the step of passing the blanks of Figure 1 through an oven, for firing of the vitreous enamel and the metallic material and the step of stacking a number of said fired blanks, one above the other.

Figure 3 is a perspective view showing the step of placing such a stack of blanks into a die to fuse together the peripheral edges of the enamel sheets to form a monolithic structure;

Figure 4 is an exploded perspective view illustrating the step of assembling several of said monolithic structures into a capacitor;

Figure 5 is a perspective view showing the step of placing an assembly as shown in Figure 4 into

a second die, with extra liquid enamel, for fusing a hermetically sealed envelope about the same;

Figure 6 is a perspective view of a completed capacitor of the stacked type after the completion of the fusing operation of Figure 5;

Figure 7 is a perspective view showing the steps of cutting a ribbon of vitreous enamel into rectangular sheets and of spraying metallic material on to each one separately, this being a modification of the step shown in Figure 1;

Figure 8 is a perspective view showing the steps of cutting a ribbon of metal foil into paddle-shaped plates and of spraying said plates, two at a time, with a thin coating of vitreous enamel;

Figure 9 is a perspective view showing the step of passing the two plate units of Figure 8 through an oven for firing of the enamel and the step of cutting them into individual blanks;

Figure 10 is a perspective view showing the step of stacking the blanks of Figure 9;

Figure 11 is a perspective view showing a modification of the spraying step of Figure 8, wherein a plurality of paddle-shaped metal plates are sprayed with vitreous enamel in one operation, and the step of passing the coated plates through a firing oven;

Figure 12 is a perspective view of another modification of the coating operation, shown in Figure 8 or 11, wherein a plurality of paddle-shaped plates of metal foil are simultaneously dipped into a bath of liquid vitreous enamel and are then passed through an oven for firing;

Figures 13 and 14 are perspective views showing diagrammatically the machine components and steps of a process for "production line" manufacture of roll type capacitors, some of the parts being omitted and others being broken away for clarity, Figure 13 showing the steps of cleaning two ribbons of metal foil, coating them with enamel, baking them, winding them into rolls and firing them, and Figure 14 showing the steps of attaching terminal wires to the rolls and hermetically sealing them within vitreous enamel envelopes;

Figure 15 is an elevational view of one of the terminal wire applicators of Figure 14, the retracted positions of the gripper and burner being shown by solid lines and the intermediate position of the gripper by broken lines;

Figure 16 is an elevational view of the tube sealer of Figure 14, the burners being shown in their operating positions and the left burner being cross-sectioned;

Figure 17 is an enlarged cross-sectional view of a rolled type capacitor, manufactured as shown in Figure 13 through 16, the left half showing the capacitor roll after the firing operation and the right half showing the finished capacitor;

Figure 18 is a perspective view showing a modification of the spraying step of Figure 13, wherein two spraying plates are substituted for a spraying tube; and

Figure 19 is a perspective view of another modification of said spraying step of Figure 13, wherein a ribbon of metal foil is dipped into a bath of liquid vitreous enamel.

In my process for the manufacture of stacked type capacitors, shown in Figures 1 through 6, a long ribbon of vitreous enamel film 51 (Figure 1), in its green state, is supported upon a flat conveyor 53 which is movable in the direction indicated by the arrow. The said conveyor, and other conveyors which will be referred to herein, may be of stainless steel or any other suitable material. Said enamel film 51 may have been

deposited on said conveyor 53 by spraying, as will hereinafter appear, or in any other suitable manner. A spraying shield 55 is superimposed over said enamel 51, said shield being provided with a plurality of paddle-shaped openings 57, equally spaced from each other. The shield 55 may be moved into place for use or it may be permanently supported slightly above the conveyor 53. The spraying shield 55 is so positioned that the extremities of the narrow tab-shaped ends 59 of the paddle-shaped openings 57 project beyond one edge 61 of the ribbon of enamel film 51. The conveyor 53 is made of inert material so that, during the metal spraying process to be described, the sprayed metal will not become bonded to the conveyor.

A fine spray of metallic, electrical conducting material 65, in liquid form, such as finely powdered silver suspended in a suitable liquid binder vehicle, is then directed at the exposed portions of the vitreous enamel 51 by means of a spray nozzle 67. Said nozzle 67 is preferably oscillating so as to distribute the material 65 evenly. When a desired thickness of metallic conducting material 65 has been deposited and the shield 55 has been removed, the vitreous enamel 51 will have a plurality of thin paddle-shaped plates 69 of metallic conducting material adhering thereto. The ribbon of enamel 51 will then be severed into a plurality of blanks 73, as indicated by the broken lines (Figure 1), by means of a cutting die 71 having a plurality of mutually parallel cutting knives 72. Each blank 73 comprises a rectangular sheet 75 of vitreous enamel, one surface of which is covered by a paddle-shaped plate 69 of metallic material, said plate being of slightly smaller area and having a tab 79 projecting beyond one edge 61 of the sheet of enamel.

The blanks 73 are then carried by the conveyor 53 through a firing oven 81 (Figure 2). The firing process may be a lengthy one and may require several ranges of heat. Thus, the oven 81 may be a very long one and the conveyor 53 may pass through it at a snail's pace. It may also be desirable to transfer the blanks 73 to another conveyor (not shown) which will carry them through the oven 81. This conveyor would be much wider so that a plurality of blanks could be placed abreast upon it to be fired simultaneously. After proper firing, the blanks 73 are carried into a chute 83 leading into a rotating stacking machine 85. The chute 83 is provided with an inwardly extending arm 84 which catches one end of each blank 73 so as to cause it to enter the chute endwise. Said stacking machine 85 is provided with a compartment 87 having the configuration of a rectangle with a narrow tab-like extension 89 at each end. The stacking machine 85 is timed to rotate so that one of the fired blanks 73 is dropped into the compartment 87 at each half turn thereof so that the rectangular sheets of enamel 75 are stacked up in register but the metallic tabs 79 of consecutive blanks 73 extend in opposite directions into the extensions 89. The arm 84 may be omitted if the stacking machine 85 is designed to stop in a position 90° removed from the position shown in Figure 2. Then the blanks 73 could slide in sideways.

After a predetermined number of said blanks 73 have been stacked, they are removed from the stacking machine 85 to a fusing die composed of two parts 91, 93 (Figure 3). Although, for clarity, only four blanks 73 are shown in Figure 3, it will be understood that any suitable

number may be stacked. In the die 91, 93 the edge portions, of the sheets of vitreous enamel 75, which extend beyond the edges of the metallic plates 89, are fused together so that the several blanks 73 are formed into a monolithic structure 97 (Figure 4) having a plurality of metallic tabs 79 protruding out at opposite ends. The exposed metallic tabs 79 at each end may then be joined together in any suitable manner, as by soldering a lead wire directly to the tabs 79 or by means of a U-shaped metal clip 99 (Figure 4) pierced by horizontal holes, and a pin or rod 101 passing through the holes of each clip and through the tabs within it and a lead wire 105 attached to said pin. Although a method using clips 99 is here shown, it will be understood that soldering a lead wire directly to the tabs 79 is a preferred construction where the metallic material has been sprayed on. Then, the tabs 79 need extend only an infinitesimal distance beyond the edge 61 of the vitreous enamel sheets 75. Also, for added strength, the tabs 79 may be as wide as the metallic plates 89 themselves. The construction shown in Figures 4 and 5 is, however, a preferred arrangement where metal foil is used for the plates, as will be referred to hereafter in connection with the processes illustrated in Figures 8 through 12.

If an entire capacitor were made of but one of the monolithic structures 97, described above, there might be a tendency for the large number of blanks 73 to buckle or warp during firing. This tendency is avoided, however, by making the monolithic structures 97 of fewer blanks 73 and then assembling a number of such structures together (Figures 4 and 5). In this construction, I find it advisable to insert stiffening sheets of vitreous enamel 103 (considerably thicker than the sheets 75 aforementioned, and preferably of the order of .01 to .03 inch), between the several monolithic structures 97 and at the top and bottom of the assembly. If the leads are soldered directly to the tabs 79, they will then be soldered to the tabs of the several structures 97 in the assembly. If the construction shown (Figures 4 and 5) is used, the pins or rods 101 will pass through the clips 99 and tabs 79 of all of the monolithic structures 97 and a lead wire 105 will be attached, by soldering or otherwise, to each of said pins. Although Figure 4 shows an assembly comprising but two of said monolithic structures 97, it will be understood that any number of them may be used. Where but one monolithic structure 97 is to be used for the finished capacitor it is advisable to place a stiffening sheet 103 above and below the stack of blanks 73 or, at least at that end of the stack which has an exposed metallic plate 69 (as the upper end in Figure 3).

The assembly just described (Figures 4 and 5) is then placed into a second fusing die (Figure 5) comprising an upper half 107 and a lower half 109. Slots 111 are provided at both ends of both die components 107, 109 to accommodate the lead wires 105. The assembly aforesaid of several monolithic structures 97 is placed into said second fusing die 107, 109 with sufficient liquid vitreous enamel 113 to completely surround it, and firing takes place so that, except for the outwardly extending lead wires 105, the finished capacitor 115 (Figure 6) is a unitary structure completely enclosed and hermetically sealed within a vitreous enamel envelope 117. Said envelope 117 is fused about the leads 105 which extend through the vitreous enamel as in a radio

tube. The enamel envelope 117 may also be dispersed about the assembly aforesaid by being sprayed thereon or by dipping the assembly into a tank of enamel or in any other suitable manner.

Although I have described the step of cutting the enamel ribbon 51 into rectangular sheets 75 (Figure 1) as taking place while the enamel is still in its green state, this may be done after firing. In that event, a ribbon of enamel film 51 with a plurality of paddle-shaped metallic plates 69 thereon (as shown in Figure 1) will be fired as a unit and will thereafter be cut so as to form blanks 73, which may then be stacked in the manner already described.

In a modified procedure for forming the blanks 73, rectangular sheets of green vitreous enamel 75 are cut or punched from ribbons 51 or larger sheets thereof by any suitable means, such as by a cutting knife 119 (Figure 7). In either case said rectangular sheets 75 may be produced in quantity by moving the vitreous enamel into place, as on a conveyor 121 (Figure 7) and dropping the rectangular sheets onto another conveyor 123. The second conveyor 123 then carries the sheets 75 into position relative to a jig of vertical guide rods 125 (Figure 7), sustained from above, so that a spraying shield 127, vertically slidably on said guide rods 125, may be dropped down over said sheet 75. The shield 127 is provided with a paddle-shaped opening 57 (as previously described above in connection with Figure 1). Metallic conducting material in liquid form 65 may then be sprayed through the shield 127 so as to form a paddle-shaped plate of metallic conducting material, the extremity of the tab of which projects beyond one edge of the rectangular sheet 75. After the steps illustrated in Figure 7, the blanks 73 resulting therefrom may then be processed as already explained, and illustrated in Figures 2 through 6.

The stacked type capacitors described above incorporate metallic, electrical conducting film, applied in liquid or paste form. A process for fabricating such capacitors, utilizing metal foil for the conducting plates, will now be set forth. In this process a long narrow ribbon of metal foil 129 is fed between guides 131 to a cutting die 133 (Figure 8) which, with each downward stroke, cuts out two paddle-shaped metal plates 135, the tabs 137 of which are oppositely disposed. Each pair of the plates 135 is then carried by conveyor 139, moving as indicated by the arrow, under a spraying shield 141 which is provided with a rectangular opening 143. The plates 135, except for the extremities 145 of the tabs 137, which are covered by the spraying shield 141, are then sprayed with liquid vitreous enamel 147 by means of a spray nozzle 149 (Figure 8). This spraying operation results in a plurality of units 151, each comprising two metal plates 135 covered, except for the extremities 145 of their tabs 137 by vitreous enamel 147. These units 151 are then passed through a firing oven 81 (Figure 9) (as already described above in connection with Figure 2). The units 151 are then fed by the conveyor 139 (Figure 9) under a cutting knife 119, which cuts each unit into two blanks 153 which are thereupon carried by another conveyor 155 to a stacking machine 157 (Figure 10), provided with a compartment 87 (as already described in connection with the rotating stacking machine 85 shown in Figure 2).

It is to be noted that, in this process, the consecutive blanks 153 are cut so as to have their projecting tabs 137 extend in opposite directions

and, therefore, the stacking machine 157 need not be of the rotating type. When a sufficient number of blanks 153 have been fed into the stacking machine 157 they are removed and fused into a monolithic structure and ultimately formed into a finished capacitor (similar to the monolithic structure 87 and the capacitor 115 described above and illustrated in Figures 3 through 6).

In a modification (Figure 11) of the process just described, paddle-shaped plates 135 of metal foil are cut out by the use of a suitable cutting die (such as the die 133 of Figure 8 or preferably, to minimize handling, a die which will cut the metallic foil so that all of the tabs 137 will extend in the same direction). After cutting, a plurality of these plates 135 are positioned on a flat surface, spaced from each other and with the tabs 137 all extending in the same direction (Figure 11). A spraying shield 159, provided with a rectangular opening 161, is positioned over a number of such plates 135 so as to cover up only the extremities 145 of their tabs 137, whereupon vitreous enamel in liquid form 147 is sprayed through the shield by means of spray nozzle 149. The shield 159 is then removed and the enamel coated plates are moved in the direction of the arrow (Figure 11) into a firing oven 81 by means of a conveyor 163, where they are fired. They may then be cut into individual blanks 153 by means of a cutting die (such as die 11 shown in Figure 1). The resulting blanks 153 are then subjected to a processing similar to that described above and illustrated in Figures 2 through 6. It is to be noted, that, if desired, the enamel coated plates 135 may first be sent through a baking oven (not shown), to bring the enamel to its green state, may then be cut into blanks 153 and may then be sent through the firing oven 81 for firing.

In another modification (Figure 12), paddle-shaped plates 135 of metallic foil are cut out (for example as shown in Figure 8). A plurality of said plates 135 are then gripped, by the extremities 145 of their tabs 137, and depended from a rack 165 (Figure 12). The rack is lowered to dip the plates 135 into a vat 167 of vitreous enamel 147 in liquid form (Figure 12) so that, except for their gripped extremities 145, said plates are completely coated with vitreous enamel. The rack 165 and enamel coated plates are then carried, as indicated by the arrow (Figure 12), by means of an intermittently moving cable 169, into a firing oven 81. The blanks 171 may then be stacked and formed into finished capacitors 115 in any suitable manner, such as is described above and illustrated in Figures 2 through 6.

It is to be noted that, in the last described modification, both surfaces of the metal foil plates 135 are coated with vitreous enamel 147. Thus, when the blanks 171 are stacked, there are two sheets of enamel dielectric 147 between consecutive metal conducting plates 135. Although this construction increases the thickness of the finished capacitor 115, it is to be strongly recommended as it precludes the possibility of electrical shorts or leakage between metal plates 135 through pin holes or air bubbles in the thin sheets of vitreous enamel 147. I have found that, although pin holes or bubbles are very infrequent, they are nevertheless possible. However, when two sheets of vitreous enamel 147 are superimposed, pin holes or bubbles in the two sheets will practically never occur in register.

By suitable modifications, coating of both sides of the metallic conducting material or metal foil may be accomplished in each of the processes

described above. Thus, in the first process set forth, after a layer of metallic conducting material 65 has been sprayed upon the ribbon of enamel 51 (Figure 1), the spraying shield 55 may be removed and a spraying shield provided with a rectangular opening (such as the shield 159, shown in Figure 11) may be substituted and a coating of liquid enamel 147 may be sprayed over the plate of metallic material 69 except for the extremity of its tab 19, thereby coating both sides of said plate. The procedure may then continue as already described.

Similarly, coating on both sides may be effectuated in the modification illustrated in Figure 7 by spraying liquid enamel 147 through a shield (not shown) with a rectangular opening after the paddle-shaped plate of metallic material has been sprayed on through the shield 127.

The metal foil plates 135 shown in Figure 8 through 11 may be coated on both sides in any of several ways. For instance, after spraying enamel on one side of the plates 135 (as illustrated in Figures 8 and 11), they may be turned over and similarly sprayed on the other side.

Enamel coating may also be applied to the under surfaces of the metal foil plates 135 (of Figures 8 and 11) by spraying said under surfaces by means of upwardly directed spraying nozzles (not shown) disposed below said plates (in a manner which will hereinafter more clearly appear in connection with the manufacture of rolled type capacitors).

There will now be described a process, according to my invention, for the fabrication of rolled type capacitors. The various steps of the process and suitable machinery to accomplish the same are diagrammatically shown in Figures 13 through 16, two modifications thereof are shown in Figures 18 and 19 and the internal make-up of a capacitor is shown in Figure 17. The capacitors are made up of two long ribbons of metal foil 173, 175. Each such ribbon is separately cleaned, coated with vitreous enamel dielectric 177 and partly baked to allow proper handling. They are then wound together about a core 179 and the resulting roll 181 is thoroughly fired. Electrical terminal wire leads 183 are then attached and the roll 181 is completely encased in a tubular envelope 185 of vitreous enamel. These steps will now be considered in detail.

For efficient manufacture, the components of the machinery to perform the various steps of the process are preferably positioned substantially linearly. Referring now to Figure 13, the sequence of the production line is shown from left to right. To the left are two horizontally disposed, freely rotatable spindles 187, one above the other, each being receivable to a spool 189, wound with a long ribbon of metal foil 173, 175. To the right of said spindles 187, also one above the other, are two rectangular tanks 191 of acid 193. Two opposite rims 195 of each tank 191 are smoothly rounded (or may be fitted with freely rotatable rollers) and, intermediate said rounded rims, is a partly submerged, smooth surfaced, cylindrical cross piece 197. A second pair of similar tanks (not shown), also one above the other, containing rinsing solution (not shown), are positioned to the right of the acid tanks 191. As may be seen in Figure 13, the spool 189 and the acid tank 191 of the lower tier are slightly nearer the observer than the corresponding components of the upper tier. The rinsing solution tanks (not shown) are similarly disposed. To the right of the tanks of rinsing solution (not shown) is a

hydrogen furnace 199 provided with two shallow horizontal slots 201 extending completely through it.

Further along to the right are two spraying tubes 203 (Figure 13), one above the other. Each tube 203 comprises a pair of flat spraying shields 205, one above the other, each such shield being provided with a rectangular spray opening 207. The shields 205 of each tube 203, are spaced slightly from each other and are joined along their lateral edges, so as to form a shallow passage 209 therebetween. Although the tubes 203 are offset, so that the lower tube and its passage 209 are slightly nearer the observer than the upper tube 203 and its passage, the four openings 207 thereof are in register. Above and below the spraying tubes 203 are four spray nozzles 211 that direct sprays of vitreous enamel 177, in liquid form, through the openings 207. To the right of the spraying tubes 203 is a baking oven 215 pierced by two shallow horizontal slots 217. The lower slots 201, 217 of both the hydrogen oven 199 and baking oven 215 are slightly nearer the observer than the upper slots thereof.

Still further to the right are four freely rotatable rollers 219 (Figure 13) and beyond them a cutter 221 provided with two cutting knives 223, one at a slightly higher level than the other. To the right of the cutter 221 is a winding device 230 (not shown) of any conventional type, which is adapted to grip and rotate a horizontally disposed cylindrical core 179.

The continuation of the production line now to be described is shown at the right in Figure 13 and from left to right in Figure 14, the parts being shown in their respective positions at an instant when the conveyors 225, 226 have just come to rest. Below the winding device aforesaid (not shown) a conveyor 225 enters the production line from below and it moves to the right through a firing and annealing oven 227 (Figures 13 and 14) pierced by a single passageway 229. Said conveyor 225 moves intermittently to the right, as indicated by the arrows, and it is provided with a plurality of two piece, substantially Y-shaped clips 231. The said firing and annealing oven 227 is of sufficient length to allow the maintenance of firing temperatures through its left portion and annealing temperatures through its right portion. If desired, two successive ovens (not shown), one for firing and the other for annealing, may be substituted for the single oven 227.

After said conveyor 225 has progressed through the oven 227, it passes between a pair (only the far one is shown) of flux applicators 233 (Figure 14), each of which is a cup 235 having within it a circular pad 237 kept saturated with soldering flux 239. Said conveyor 225 then passes between a pair (only the far one is shown) of solder applicators 241, each of which is an electrically heated cup 243 to which solder 245 is automatically fed. Said flux applicators 233 and solder applicators 241 are movable, horizontally, toward and away from the conveyor 225, as indicated by the arrows. They are normally in their retracted positions but, each time a clip 231 on the conveyor 225 comes to rest between them, they move inwardly toward the conveyor to perform their respective operations and they then return to their normal positions.

Further to the right the conveyor 225 passes between a pair of terminal wire applicators 247 (Figures 14 and 15). Each of such applicators 247 includes a gripper 249 which is normally in

a retracted position (shown in solid lines in Figures 14 and 15) and is adapted to grip a horizontally disposed lead-in wire 183, move it toward the conveyor 225, release said wire and then return to its normal position. Positioned directly above each gripper 249, when in its retracted position, is a vertically disposed, stationary, T-shaped chute 251 (Figures 14 and 15) adapted to hold a column of terminal wires 183. The lower end of each chute 251 is provided with a closure (not shown) which is opened momentarily, each time the gripper moves back to its retracted position, to release one terminal wire 183 and drop it into the gripper 249 below it. Said closure opens when an upwardly extending pin 253 on the gripper 249 actuates a depending finger 255 on the chute 251. Each terminal wire 183 in the chute 251 comprises a length of wire 257 terminating in a metal disk 259 having a rounded back and a flat face, which has been previously tinned for soldering.

Encircling the horizontal axis of movement of each gripper 249 is a vertically disposed ring-shaped burner 261 which convergently directs several small flames 263 in the direction of the conveyor 225. Said burner 261 is also normally in its retracted position (as shown in solid lines in Figures 14 and 15), but moves inwardly with the gripper 249, after the gripper has passed beyond its intermediate position (shown in broken lines in Figure 15) and then said burner returns to its retracted position.

Further to the right and positioned at the far side of said conveyor 225 is a tube conveyor 226 (Figure 14), movable intermittently to the right as indicated by the arrow, in synchronism with the movements of said conveyor 225. Extending upward from the said tube conveyor 226 are a plurality of U-shaped tube holders 265, the leading edge of each such holder being provided with an upwardly extending arm 267. Above said conveyor 226 is a stationary, vertically disposed, rectangular tube chute 269 accommodating a plurality of cylindrical vitreous enamel tubes 185. Each tube 185 is of a diameter to allow a capacitor roll 181 to be slid within it and of a length greater than such capacitor roll. The lower end of the tube chute 269 is provided with a suitable closure (not shown) and latch 271 which allows the discharge of one tube 185 each time a tube holder 265 moves into position below said tube chute. Said closure is opened by coaction between the arm 267 and the latch 271. The far wall 272 of said chute extends down to about the level of the tube conveyor 226 and is partly cut by a horizontal slot 270.

On the near side of the conveyor 225, opposite the tube chute 269 is a pusher rod 273 (Figure 14), comprising a vertical ring affixed to the end of a horizontal rod, which is normally in a retracted position (as shown in Figure 14) but which is caused to move horizontally, as indicated by the arrow, across the conveyor 225 toward the tube conveyor 226, each time said conveyors 225, 226 come to rest, and then to return to its retracted position.

The tube conveyor 226 extends horizontally for a short distance to the right and then drops downward to a lower level where it again continues on to the right. Just beyond the drop is located a tube sealer 274 (Figures 14 and 16), which includes a pair of mutually parallel rollers 275, 276 and a pair of burners 277. The rollers 275, 276 are disposed transversely above the tube conveyor 226 and are so spaced as to support

one of the vitreous enamel tubes 185 aforesaid. The left roller 275 is rotated by any conventional means (not shown) so as to cause a tube supported thereon to spin about its axis. The right roller 276 is freely rotatable and it also moves downwardly and to the left a short distance each time the burners 277 return from their operating to their retracted positions, as will now be described. Flanking the tube conveyor 226, abreast of said rollers 275, are two, vertically disposed, horizontally movable, ring-shaped burners 277 (see Figure 14, which shows only the far burner, and Figure 16), each of which convergently directs needle-pointed flames 279 inwardly. Said burners 277 are normally in retracted positions (as in Figure 14) but move inwardly to their operating positions (Figure 16) each time the tube conveyor 226 comes to rest, to direct their flames 279 at the ends of a spinning tube 185 and then return to their retracted positions. While in their operating positions, said burners 277 oscillate several times a short distance in and out. To the right of the rollers 275, 276 the tube conveyor 226 passes through an annealing oven 281, which is provided with a horizontal through passageway (not shown).

A process for the manufacture of roll type capacitors, according to my invention and utilizing the machinery components already described and shown in Figures 13 through 16, is as follows:

Referring to Figure 13, the ribbon of metal foil 173 on the upper spool 189 is threaded over the left rim 195, under the rounded cross-piece 197 and over the right rim 195, of the upper tank 191 of acid 193 and is similarly threaded through the second upper tank of rinsing solution (not shown). It is also threaded through the upper slot 201 of the hydrogen furnace 199, through the passage 209 of the upper spraying tube 203 and through the upper slot 211 of the baking oven 215. From the baking oven 215 it extends successively over and under the two upper rollers 219 and under the upper cutting knife 223 of the cutter 221.

The ribbon of metal foil 175 on the lower spool 189 extends, in a similar manner, through the lower tier of all of the components just described. The ends of the two ribbons of foil 173, 175, after extending through the cutter 221, are wound about the core 179, the first couple of turns having been wound on by hand or by a suitable mechanism (not shown).

In operation, the winding device (not shown) will rotate at a steady speed and will pull the two ribbons of metal foil 173, 175, in the direction indicated by the arrow, successively through the various components just mentioned. The metal foil will be suitably cleaned in passing through the baths of acid 193 and rinsing solution and the hydrogen furnace 199. These three steps are intended to free the metal foils 173, 175 of any oxides, chemicals, grease, dirt and impurities which might interfere with the subsequent steps of manufacture or which might detract from the efficiency of the finished capacitor. The order of these cleaning steps may be rearranged or one or more omitted or other cleaning means included, as may be found best for the particular materials being used and the condition thereof.

In passing through the spraying tubes 203 both the upper and lower surfaces of both ribbons of metal foil 173, 175 will be sprayed with a thin coating of vitreous enamel 177. It will be noted, however, that a narrow strip 283 of metal foil along the far edge of the upper ribbon 173 and

a narrow strip 285 of metal foil along the near edge of the lower ribbon 175 will be left uncoated, in view of the fact that, as already described, the passages 209 are offset in opposite lateral directions relative to the spray openings 207. The speed of movement of the foils 173, 175, the lengths of the spray openings 207 and the quantity of enamel 177 being sprayed will be so adjusted that the enamel coating will be of a predetermined thickness.

The enamel coated foils 173, 175 are then pulled through the baking oven 215, the length of the oven and its temperature being such that the vitreous enamel 177 is given a partial baking until it reaches its "green" state. Said coated foils 173, 175 are then brought into closer proximity by means of the rollers 219 and they then pass through the cutter 221 and around the core 179. They reach the core 179 in superimposed relationship, except that the uncoated strips 283, 285 extend outwardly laterally in opposite directions. When the winding device has wound predetermined lengths of the enamel coated foils 173, 175, about the core 179, to form a capacitor roll 181, the two cutting knives 223 operate so as to sever said foils.

The capacitor roll 181 is then removed from the winding device, either manually or by a suitable mechanism (not shown), and dropped into one of the Y-shaped clips 231 of the conveyor 225 which carries it through the firing and annealing oven 227. There the vitreous enamel 177 is thoroughly fired so that contiguous layers of enamel fuse together and the capacitor roll 181 becomes a monolithic structure, its internal make-up at that stage being as shown in the left half of Figure 17. The length of the oven 227, the temperatures maintained in the left and right portions thereof and the speed of the conveyor 225 are such as to fire and anneal the vitreous enamel dielectric 177 of the roll 181 according to a predetermined formula. As already mentioned above, in connection with stacked type capacitors, the oven 227 may be provided with a much wider conveyor (not shown) running at a very slow rate upon which a number of capacitor rolls 181 may be placed abreast. After coming out of the oven 227 upon such a conveyor the rolls 181 would be transferred, manually or by suitable apparatus, to the conveyor 225 for continuation of their processing. The conveyor 225 moves intermittently and carries several capacitor rolls 181, so that, after being fired, each roll is moved successively to various positions, at each of which it is brought to rest and is partly processed. Hence, several capacitor rolls 181 which are positioned along the conveyor 225 at any one time are simultaneously subjected to processing operations, succeeding rolls however undergoing succeeding processing steps.

When a capacitor roll 181 is brought to rest between the two flux applicators 233, said applicators, which are normally retracted (as in Figure 14), move inwardly simultaneously against the opposite ends of the capacitor roll, the roll being held above the level of the conveyor 225 by one of the clips 231. The pads 237 of said flux applicators 233 crumple the uncoated strips 283, 285 of metal foil against the opposite ends of the roll 181 and also apply soldering flux 239 thereto. Said flux applicators 233 then retract and the conveyor 225 moves the roll 181 to a position intermediate the two solder applicators 241, which move inwardly simultaneously and respectively apply suitable predetermined charges of solder

245 to the crumpled strips 283, 285 of foil at both ends of the roll.

Said solder applicators 241 then retract and the roll 181 is moved on to a position between the two terminal wire applicators 247. Each gripper 249 is then in its normal retracted position (shown by solid lines in Figures 14 and 15) and a terminal wire 183 has already been dropped into it (by coaction between pin 253 and finger 255 on the previous outward return stroke of said gripper). The two grippers 249 then move inwardly simultaneously until they reach their intermediate positions (shown by broken lines in Figure 15) at which point the flames 263 will play upon the disks 259 of the terminal wires 183. The grippers 249 and their associated burners 261 then move inwardly together, the flames 263 continuing to heat the disks 259, until the flat faces of the disks abut against the crumpled strips 283, 285. After a short interval, predetermined as being necessary to effect soldered connections between said disks 259 and strips 283, 285, the burners move back to their retracted positions and then the grippers 249 release their respective terminal wires 183 and the burners return to their normal retracted positions, another terminal wire being discharged from each chute 251 and dropped into each gripper at the end of its outward stroke.

The conveyor 225 moves the roll 181, now fitted with a terminal wire 183 at each end, into position opposite the tube chute 269. As it reaches that position, coaction between one of the arms 267 and the latch 271 causes the lowermost enamel tube 185 in said chute to drop into one of the tube holders 265 on the tube conveyor 226. The pusher rod 273 then moves inwardly from the near side of the conveyor 225 and propels the roll 181 into the said tube 185. The far wall 272 of said tube chute 269 keeps the tube 185 in position during this operation. The pusher rod 273, being ring-shaped, does not interfere with the near terminal wire 183. If the conveyors 225, 226 are too far apart, it may be advisable to position a stationary trough (not shown) between the conveyor 225 and the tube conveyor 226 to help guide each roll 181 into a tube 185.

When a tube 185, with a capacitor roll 181 within it, reaches the point where the conveyor 226 drops downward, said tube falls into position upon the rollers 275, 276 whereupon it is caused to spin about its axis by the rotating roller 275. The two ring-shaped burners 277 move inwardly from their retracted positions (Figure 14) to their operating positions (Figure 16) so that the needle-pointed flames 279 play upon the ends of the spinning tube 185. Said burners 277 automatically oscillate in and out several times so that the ends of the enamel tube 185, which extend beyond the disks 259, are thoroughly heated throughout and they bend inwardly, curve about the rounded backs of the disks 259 and fuse about the terminal wires 183 so as to take the shape shown in the right half of Figure 17. The flames 279 are purposely needle-pointed so that they concentrate heat on the tube 185 but do not melt the solder 245. By the oscillation of the burners 277 and the spinning of the tube 185, an even temperature is maintained and breakage of the tube is prevented. The burners 277 then retract and the right hand rollers 276 move to its depressed position, already described, causing the capacitor roll 181 to roll over said roller into one of the holders 265 which carries it through the annealing oven 281, which anneals the tubular envelope 185. When it leaves said oven 281 it is a finished

capacitor 287 (as shown at the right half of Figure 17).

The manufacturing operations up to and including the winding of the capacitor rolls 181 (as shown in Figure 13) may not be performed with sufficient rapidity to keep the balance of the production line (shown in Figure 14) operating at its maximum capacity. Hence, it is to be understood that two or more complete sets of apparatus (as shown in Figure 13) may be operated simultaneously so as to produce sufficient capacitor rolls 181 to feed one conveyor 225.

The spraying step described above and illustrated in Figure 13 may be modified as shown in Figure 18, where it is illustrated in use with the upper ribbon of foil 173. In this modification two vertically disposed, coplanar, spraying plates 289 are substituted for each of the spraying tubes 283. Said plates 289 are spaced apart just enough to allow the ribbon of metal foil 173 to pass therebetween and they are positioned slightly in from one edge of the foil. Spray nozzles 211 above and below the foil 173 will, therefore, coat both surfaces thereof with citreous enamel 177 except for a narrow strip 283 along one edge thereof.

Another modification of the spraying step of Figure 13 is illustrated in Figure 19. Here a ribbon of metal foil 173, suspended from an elongated rack 291, is dipped, except for a narrow strip 283 along its upper edge, into a vat 293 of vitreous enamel 177 in liquid form.

Still another modification of the spraying operation of Figure 13 consists in substituting for the two spraying tubes 283 two tanks of vitreous enamel (not shown), one above the other, and two wipers (not shown), also one above the other. Each of the metal foils 173, 175 is caused to dip into one of said tanks so as to become completely coated with enamel. After leaving the tanks, each foil 173, 175 passes through a wiper which wipes off the enamel along one edge so as to leave an uncoated strip of foil 282, 295, similar to such strips as already described.

Although I have described herein a number of manufacturing processes for the production of several types of capacitors, and have described mechanisms for carrying them out, it is to be understood that the various manufacturing steps and processes described may be grouped into other combinations within the spirit and teaching of the present invention. For instance, a process for manufacturing rolled type capacitors, by spraying or otherwise applying metallic material in liquid or paste form, may be a combination of steps already described and illustrated in Figure 1 and the process described above and illustrated in Figures 13 and 14. This could be accomplished by laying down a long thin strip of enamel, by spraying or otherwise, then covering it with a long thin strip of metallic conducting material, by spraying or otherwise, one edge of said metallic strip, extending beyond the enamel, and then laying down another layer of enamel in register with the first strip of enamel. Two of these elongated laminated structures would be partially baked and then rolled together. The roll would then be placed on conveyor 225 and further processed as already described and illustrated in Figures 13 and 14.

Another modification might be made in connection with the process already described and illustrated in Figures 1 through 6. This would comprise the steps of dispersing a thin ribbon of vitreous enamel dielectric material 51, in paste or liquid form, as by spraying, and then dispers-

ing thereon a plurality of thin paddle-shaped plates 68 of metallic conducting material, in paste or liquid form, as by spraying. The ribbon 51 and the plates 68 would then be partially dried, as in a baking oven, until the enamel reached its green stage. The ribbon of enamel 51 would then be cut (as in Figure 1) to form blanks 18 which would then be stacked (as in Figure 2) and the stack of blanks would then be fired, as in a firing oven 81 (Figure 2). This would result in a monolithic structure 91 (Figure 4), which would be assembled into a finished capacitor 118 (as shown in Figures 4 through 6). It is to be noted that this modified process differs, from the process of Figures 1 through 6, in that the steps of drying the enamel 51 and spraying the metallic material 68 are reversed, the steps of firing and stacking are also reversed and the fusing step (Figure 3) is omitted entirely.

The vitreous enamel to be used in the capacitors described in the present specification should have a melting point lower than the metal foil to be used, so that the enamel may be fired without melting the foil. Also it should be of a type which has good thermal shock resistance in addition to the electrical characteristics already set forth. Some of the silicate flint glasses, such as Schott, heavy silicate flint (International Critical Tables, volume 2, 1927, index number 102), might be used, but with modifications in the formulae, better electrical characteristics may be obtained. Also, the vitreous enamel used should preferably have substantially the same coefficient of expansion as the metal parts used so as to avoid breakage of the enamel due to temperature changes, both during manufacture and in use.

What is claimed is:

1. A method of producing a rolled type capacitor consisting of dispersing a thin elongated sheet of vitreous enamel dielectric material, in liquid or paste form; dispersing a thin ribbon of metallic conducting material, in liquid or paste form, over said sheet, one edge of said ribbon extending in from one edge of said sheet and the other edge of said ribbon extending beyond the other edge of said sheet; dispersing a second sheet of vitreous enamel dielectric material, in liquid or paste form, over said first mentioned sheet and said ribbon, said second sheet being in substantial lateral register with said first mentioned sheet; partially drying said sheets and ribbon so as to form a flexible three-ply structure; forming a second similar three-ply laminated structure by the steps aforesaid; superimposing one of said laminated structures over the other so that the sheets of dielectric material are in substantial lateral register and the ribbons of conducting material are offset laterally in opposite directions; winding said laminated structures together to form a roll; firing said roll into a monolithic structure; and connecting electrical leads to said ribbons.

2. A method of producing a rolled type capacitor consisting of dispersing a thin elongated sheet of vitreous enamel dielectric material, in liquid or paste form; dispersing a thin elongated plate of metallic conducting material, in liquid or paste form, over said sheet, one lateral edge of said plate extending in from one lateral edge of said sheet and the other lateral edge of said plate extending beyond the other lateral edge of said sheet; dispersing a second thin elongated sheet of vitreous enamel dielectric material, in liquid or paste form, over said first mentioned sheet and said plate, in substantial lateral regis-

ter with said first mentioned sheet; partially drying said sheets and plate so as to form a flexible three-ply laminated structure; forming a second similar three-ply laminated structure by the steps aforesaid; superimposing one of said laminated structures over the other so that the sheets of dielectric material are in substantial lateral register and the plates of conducting material are offset laterally in opposite directions; winding said laminated structures together to form a roll; firing said roll into a monolithic structure; connecting electrical leads to said plates; dispersing a coating of vitreous enamel dielectric material about said monolithic structure and parts of said leads; and firing said coating to form a hermetically sealed envelope about the monolithic structure and the coated parts of the leads.

KRISTIAN H. BRANDT.

## REFERENCES CITED

The following references are of record in the file of this patent:

## UNITED STATES PATENTS

| Number       | Name       | Date          |
|--------------|------------|---------------|
| 425,020      | Buchanan   | Apr. 8, 1890  |
| 1,307,341    | Brinton    | June 24, 1919 |
| 1,650,395    | Siegel     | Nov. 22, 1927 |
| 10 1,721,503 | Priess     | July 23, 1929 |
| 1,745,400    | Brennecke  | Feb. 4, 1930  |
| 1,785,479    | Dubilier   | Dec. 16, 1930 |
| 1,870,949    | Dubilier   | Aug. 9, 1932  |
| 1,892,755    | Scheppmann | Jan. 3, 1933  |
| 15 2,238,031 | Brennan    | Apr. 15, 1941 |
| 2,368,458    | Engle      | Jan. 30, 1945 |
| 2,387,759    | Jarvis     | Oct. 30, 1945 |
| 2,389,420    | Deyrup     | Nov. 20, 1945 |
| 2,395,442    | Ballard    | Feb. 28, 1946 |
| 20 2,399,313 | Ballard    | Apr. 30, 1946 |